

Patented Apr. 6, 1926.

1,579,872

# UNITED STATES PATENT OFFICE.

JOSEF LECJAKY, OF NEW YORK, N. Y., ASSIGNOR TO JOSEPH SEC, OF NEW YORK, N. Y.

## MARBLEIZING PAPER.

No Drawing.

Application filed March 15, 1924. Serial No. 699,563.

To all whom it may concern:

Be it known that I, JOSEF LECJAKY, a citizen of the Czechoslovak Republic, and resident of New York city, in the county of New York and State of New York, have invented certain new and useful Improvements in Marbleizing Paper, of which the following is a specification.

The object of the present invention is to provide an improved method of marbleizing paper, and by the term "marbleizing" I mean the application of one or more colors to the paper in such manner as to produce the varied color distribution on the paper characteristic of, or analogous to that possessed by ordinary marbled or mottled papers.

My novel method is broadly characterized by the treatment of the paper with two liquid agents, one or both of which contains coloring matter of a desired color, by first coating the surface in a substantially uniform manner with one of the liquid agents and then, before this coating dries, applying the second agent to the surface at localized points thereof, the two agents being of such a character that they react chemically as distinguished from a mere dissolving effect, to spread or draw the color over the paper and thereby vary the color distribution over the portions of the paper wet by the two agents. When each of the agents contains coloring matter different from that in the other, a two-color effect is obtained. A multiple color effect can also be obtained by the application at localized points of two or more different liquid agents each containing a different coloring matter.

In a simple practical mode of carrying out the present invention of marbleizing a paper sheet, the sheet is supported on a table and has its upper surface wet in a substantially uniform manner by a walnut crystal solution containing a non-acid aniline or tar dye, applied by means of a sponge or brushes, and then a solution of potassium hydrate is sprayed onto the wetted paper. Each drop of potassium hydrate thus sprayed onto the paper spreads, and in spreading carries with it more or less of the coloring matter in the coating first applied to the paper, thus producing a characteristic marbled effect, the marble tracings thus formed varying accordingly as the supporting table is horizontal or inclined. Practically any paper containing not more than

20% or 30% of mechanical wood pulp can be marbleized in accordance with the present invention, but the paper should be thoroughly sized before being marbleized. The marbleized paper may be originally white, or of any other color not too dark to unduly obscure the marbleizing effect. When the paper is thus already colored the number of colors in the finished product is correspondingly increased.

The walnut crystals mentioned above are formed by boiling the carbonaceous humic acid containing material known as "Cassel brown", in a 40% solution of potassium carbonate or sodium hydrate in water, to evaporate the water in the solution. The walnut crystal solution is formed by adding to water from 1% to 5% of walnut crystals, decanting the solution thereby formed, and adding ordinarily from 1% to 5% of powdered or crystallin non-acid aniline or tar dye of the desired color. Practically any non-acid aniline or tar dye soluble in water may be used, and the quantity of the dye employed depends upon the effectiveness of the dye and the intensity of color desired. The potassium hydrate solution employed is of the strength obtained by dissolving from 2½ to 10 grammes of potassium hydrate in a liter of water.

In lieu of potassium hydrate as the agent applied to distributed points of the paper surface still wet by the walnut crystal solution, I may employ other saline solutions, as solutions of potassium carbonate, potassium phosphate ( $K_2HPO_4$ ), sodium hydrate, sodium carbonate and sodium phosphate ( $Na_2HPO_4$ ) act in about the same way as potassium hydrate when used as above described, except that with the sodium or potassium phosphate solutions larger marble spots are produced.

In lieu of spraying the color wet paper with a solution which, like those above specified, tend to disperse the color, I may spray the wet paper with a solution of Roman alum ( $(SO_4)_2AlK$ ), which tends to concentrate the color and produce a sort of starred effect.

Whether the material sprayed on the color wet paper has a color dispersing effect as does potassium hydrate, or a color concentrating effect as does Roman alum, the material sprayed may itself contain a suitable non-acid aniline or tar dye thus giving a double color marble effect.

The general principles of the invention as above described may be employed in modified form or in conjunction with additional steps to produce somewhat different 5 effects. For example, to produce a "fluss" or river marble effect, the paper is first coated with a walnut crystal dye containing solution, and the localized application of potassium hydrate or analogous solution is 10 made by dabbing it on the surface of the paper with a small sponge. In this case the walnut crystal solution first applied is advantageously of the strength obtained by dissolving from 50 to 70 grammes of walnut 15 crystals in a liter of water.

In producing the so-called "mottled" or cloud papers covered with two, or three, or more colors, I advantageously proceed by first coating the paper as before with a 20 walnut crystal solution containing the basic color dye, which in this case must obviously be of a relatively light shade, and then spray the wetted surface with an additional coloring agent, or spray it successively with two 25 or more additional color containing liquids, after which I spray the paper with the saline color spreading agent, which in this case is preferably sodium or potassium phosphate rather than the other sodium and potassium 30 containing substances mentioned above. The additional color containing liquid or liquids used in this form of the invention are preferably each formed by adding a non-acid aniline or tar dye of the desired color to a 35 solution formed by dissolving walnut crystals and hard soap in water, the constituents of the solution being in or about the ratio of 10 parts of walnut crystals, 10 parts of dye, 1 to 2 parts of hard soap and 40 1,000 parts of water. The quantity of hard soap specified is based on the assumption that the soap is dry. The excess fat in the hard soap enhances the color distributing effect of the reaction between the other 45 agents employed.

In lieu of first coating the paper with a walnut crystal solution and thereafter spraying the wetted surface with a saline agent reacting with the walnut crystal solution to 50 spread the color, I may first wet the paper uniformly with the saline agent and then spray the wetted surface with the walnut crystal solution. In preparing mottled papers with this reversal of steps, the saline 55 agent may well be a sodium phosphate solution of the strength formed by dissolving 10 parts of sodium phosphate in 1,000 parts of water and the walnut crystal solution sprayed on the wetted surface may advantageously be formed by dissolving 50 parts of walnut crystals, and at least 50 parts of a

non-acid aniline or coal tar dye of relatively strong coloring, and from 2 to 7 parts of hard soap, in 1,000 parts of water.

I may use a solution of potassium or 65 sodium hydroxide instead of a walnut crystal solution and secure somewhat the same effects as are obtained by proceeding in the modes above described, but I prefer the use of the walnut crystal solutions, as 70 such a solution forms a good mordant and the color of the undyed walnut crystal solution is ordinarily beneficial rather than otherwise so far as the ultimate color effect produced is concerned. Moreover, the colors 75 produced when the walnut crystal solutions are employed after once drying are practically water proof, probably due to the presence of humic acid in Cassel brown, whereas when the walnut crystal solution is 80 replaced by a solution of potassium or sodium hydrate, the dried color effects produced are not water proof and the colored papers must be shellacked or otherwise treated to make them water proof. 85

Having now described my invention, what I claim as new and desire to secure by Letters Patent, is:

1. The method of marbleizing a paper surface which consists in coating the surface with one liquid agent and then, before the coating dries, applying a second liquid agent to said surface at localized points thereof, one or both of said agents containing coloring matter and one of said agents including 90 a small quantity of hard soap and the two agents chemically co-operating to vary the distribution of said coloring matter on the portions of the surface wetted by both of 95 said agents.

2. The method of marbleizing a paper surface by means of two liquid agents, one of which is a walnut crystal solution while the other is a saline solution and one or both of which contains a non-acid aniline or coal 100 tar dye, by first wetting said surface with one of said agents and then applying the other agent to said surface at localized 105 points thereof.

3. The method of marbleizing paper 110 which consists in wetting the surface of the paper with a colored walnut crystal solution, spraying onto the wetted paper a second walnut crystal solution of a different color and containing dissolved hard soap, 115 and finally spraying the paper with a potassium or sodium phosphate solution.

Signed at New York city, in the county of New York and State of New York, this 14th day of March, A. D. 1924.

JOSEF LECJAKY.